

# United States Patent Office

2,695,833

Patented Nov. 30, 1954

1

2,695,833

## PROCESS FOR MAKING FLAMEPROOFED DYED AMINIZED COTTON FABRICS

Oscar J. McMillan, Jr., and John D. Guthrie, New Orleans, La., assignors to the United States of America as represented by the Secretary of Agriculture

No Drawing. Application May 9, 1952,  
Serial No. 287,025

4 Claims. (Cl. 8—57)

(Granted under Title 35, U. S. Code (1952), sec. 266)

A non-exclusive, irrevocable, royalty-free license in the invention herein described, for all governmental purposes, throughout the world, with the power to grant sub-licenses for such purposes, is hereby granted to the Government of the United States of America.

This invention relates to reducing the combustibility of materials composed essentially of cellulose fibers, particularly cotton fabrics. More particularly this invention provides a process of producing deeply colored cotton fabrics of low combustibility.

We have discovered that cotton fabrics can be aminized and dyed to produce deeply colored fabrics of low combustibility. We have further discovered that such fabrics can be impregnated with poly(triallyl phosphate) to produce deeply colored fabrics having a hand and feel adapting them for the conventional uses of deeply colored fabrics, having a marked resistance to changes in flammability due to washing, and having flammability properties enabling them to pass the American Association of Textile Chemists and Colorists Standard Test Method 3437 Vertical Flame Test.

In general, according to this invention, materials composed of cellulose fibers, preferably cotton fabrics, are converted to deeply colored fabrics of low combustibility by: aminizing them until they have an amine nitrogen content of at least about 0.6% and dyeing them with an acid reacting azo dye containing at least one radical of the group consisting of phosphato and sulfo radicals until at least 7% of the weight of the dyed fabric is dyestuff. Deeply dyed fabrics which will pass the above vertical flame test are produced by: aminizing and dyeing cotton fabrics in the same way; impregnating the dyed fabrics with a solution of poly(triallyl phosphate) until at least 10% poly(triallyl phosphate) is dispersed throughout the interstices of the fabric; and removing the solvent and curing the fabric.

While the cotton fabric can suitably be aminized by a variety of known methods, the fabric is preferably aminized by aminoethylation, for example by the process described in U. S. 2,459,222. While the aminization can suitably be conducted to produce aminized fabrics containing a substantially greater proportion of amino nitrogen, an aminization to an amino nitrogen content of greater than about 1% markedly increases the boardyness of the fabric.

Substantially any acid reacting azo dye containing at least one radical of the group consisting of phosphato and sulfo radicals can suitably be used. Preferred dyes include the phosphorous containing dyes described in U. S. 2,183,998 and the sulfur containing dyes described in the colour index published by the Society of Dyers and Colourists of Great Britain. Direct cotton dyes are particularly suitable in that their use results in a particularly high retention of the property of low flammability after launderings and the like treatments. Particularly suitable dyes include those commercially available under the trade names: Kiton Fast Red; Kiton Fast Yellow; Kiton Red S; Kiton Blue A; Kiton Red G; Kiton Red 6B; Kiton Fast Orange G; Kiton Fast Green V; Kiton Fast Violet 10B; Amacid Light Yellow 2G; Amacid Brilliant Orange; National Diazine Black H; Pontamine Fast Blue 4G LN; National Erie Yellow F; Pontamine Sky Blue 6BX; Pontamine Fast Pink BL.

While the aminized cotton fabric can suitably be dyed until substantially more than about 7% of the weight of the dyed fabric is pure dye, little advantage is provided

2

by the presence of the additional amount, and dyeing until about 7% of the weight of the dyed fabric is dyestuff is preferred. In practice, due to the fact that commercial dyes are seldom pure, about 10 percent or more of commercial dyes, based on the weight of the fabric, is used.

The dyeing can suitably be conducted in accordance with the conventional processes of dyeing amino group-containing fabrics. Wool dyes are preferably applied in an acid medium, and aqueous mediums made acid with acetic acid are particularly suitable. Direct cotton dyes are preferably applied in an aqueous medium which is initially slightly basic and which is rendered acidic by the addition of acetic acid. The dyeing is preferably aided by the addition of salt to the aqueous medium containing the dye, toward the end of the dyeing operation.

The poly(triallyl phosphate) used in the process of this invention can suitably be a liquid polymer or a solid polymer which is appreciably soluble in some volatile organic solvent. Suitable methods of preparing triallyl phosphate are described in U. S. 2,394,829. Polymerization is accomplished by known methods using a peroxide, for example, benzoyl peroxide, as a catalyst. While the poly(triallyl phosphate) can suitably be applied to the dyed aminized fabric in the form of a solution in substantially any relatively volatile organic solvent for poly(triallyl phosphate) a particularly suitable solvent for such use is the methyl alcohol-ethylene chloride azeotrope boiling at about 61° C. The solution of poly(triallyl phosphate) is preferably one which contains from about 3 to about 15 percent poly(triallyl phosphate).

The aminized dyed fabric can suitably be impregnated with amounts of poly(triallyl phosphate) substantially greater or less than about 10%. However, the use of substantially less results in a lesser degree of flameproofing and the use of substantially more results in a greater degree of stiffness of the fabric.

The poly(triallyl phosphate) impregnated fabric can suitably be cured by the conventional processes for curing a chemically impregnated cotton fabric, i. e. in general from about 80° to about 130° C. for from about 60 to about 20 minutes using a longer time with a lower temperature.

The following examples are illustrative of the invention:

### Example 1

8 g. of aminized cotton fabric, consisting of 48 x 48 sheeting that had been aminoethylated according to U. S. Patent 2,459,222 and which contained 0.8 percent amino nitrogen, was placed in a dye bath containing 4 g. of Kiton Fast Red dissolved in 1 percent acetic acid. After boiling the fabric in this dye bath for about 30 minutes, the fabric was air dried. It was a very dark shade of red, and at least about 10% of its weight was the dyestuff employed.

When a 1 cm. strip of the fabric was held at an angle of 135° from the vertical and lighted at the lower end, the fabric strip did not support combustion. The undyed aminized fabric burned completely when lighted in this position and also burned completely when the strip was held with the edge at an angle of 45° from the vertical and lighted at the upper corner.

### Example 2

2 g. of a similar aminized cotton fabric containing 0.8 percent nitrogen was placed in a dye bath composed of 0.25 g. of Kiton Red 6B (sodium salt of p-acetylaminobenzene - azo - 8 - acetylaminol - 1 - naphthol - 3:6 - di-sulphonic acid), 500 ml. of water and 5 ml. of acetic acid and boiled for 1 hour. The fabric was removed from the bath and air dried. It was a dark shade of red and at least about 10% of its weight was the dyestuff employed.

The flame-resistance of the dyed fabric was similar to that described for the fabric dyed according to Example No. 1.

### Example 3

5 g. of a similar aminized cotton fabric containing 0.8 percent nitrogen was placed in a dye bath composed of

1 g. National Diazine Black H (sodium salt of diphenyl-disazo - 3 - sulpho - 7 - amino - 1 - naphthol - 8 - amino-1-naphthol-3:6-disulphonic acid), 1 g. sodium carbonate and 500 ml. water. After boiling for 30 min., 2 ml. of acetic acid was added, and the boiling continued for 30 min. more. The fabric was then washed in dilute acetic acid solution and air dried. It was a dark shade of black and at least about 10% of its weight was the dyestuff used.

The dyed fabric did not support combustion when lighted in the 135° position as described in Example No. 1.

*Example 4*

53 g. of a similar aminated fabric containing 0.8 percent nitrogen was dyed in a bath composed of 7 g. of Pontamine Fast Pink BL conc. 125% (sodium salt of 3:3' - disulphodiphenyl - urea - 4:4' - disazo - bis - 2-amino-8-naphthol-6-sulphonic acid), 7 g. of Na<sub>2</sub>CO<sub>3</sub> and 1500 ml. of distilled water at the boil for 30 min. Glacial acetic acid, 10 ml., was then added dropwise and the boiling continued for 30 min. followed by the addition of 20 g. Na<sub>2</sub>SO<sub>4</sub> and 30 min. more boiling.

After thorough washing in water and air drying the dyed fabric was a very dark red, contained about 8% of the pure dyestuff based on sulfur analysis of the fabric, and showed some flame-resistance, failing to support combustion when a strip was held at an angle of 90° from the vertical and lighted at the end.

A 3.8 percent solution of polymerized triallyl phosphate in 68% ethylene chloride and 32% methanol was applied to both sides of the fabric, allowing partial drying between each application. After air drying the fabric was baked for 1 hr. at 100° C. The fabric was thus impregnated with about 15% of the polymer.

The fabric was washed twice in a beaker with 0.1% Igepon T solution at 60° C. for 5 minutes for each wash, followed by two 5 minute washes in tap water at 60° C.

This was followed by a fluoride laundry sour after which the fabric was washed thoroughly in water and air dried.

5 The polymer-impregnated dyed fabric did not support combustion when a strip was held in a vertical position and lighted from the bottom. There was no afterglow. It passed the vertical flame test of the American Association of Textile Chemists and Colorists, Standard Test Method 34-37. In this test the char length was 3.75 inches and the fabric weight was 7 oz. per square yard. The fabric contained by analysis 1.08% nitrogen, 2.14% phosphorus and 0.93% sulfur. The dyed fabric prior to application of the polymerized triallyl phosphate contained 1.39% nitrogen, 1.13% sulfur and no phosphorus.

We claim:

1. A process of producing a deeply dyed cotton fabric of relatively low combustibility, which comprises, amino-ethylating the fabric to an amino nitrogen content of at least about 0.6% and dyeing the aminated fabric with an acid reacting azo dye containing at least one radical of the group consisting of phosphato and sulfo radicals until at least about 7% of the weight of the resulting dyed aminated fabric is dyestuff.
2. The process of claim 1 in which the dye is a sodium salt of p-acetylamo benzene-azo-8-acetylamo-1-naphthol-3:6-disulphonic acid.
3. The process of claim 1 in which the dye is a sodium salt of diphenyl-disazo - 3 - sulpho-7-amino-1-naphthol-8-amino-1-naphthol-3:6-disulphonic acid.
4. The process of claim 1 in which the dye is a sodium salt of 3:3'-disulphodiphenyl-urea-4:4'-disazo-bis-2-amino-8-naphthol-6-sulphonic acid.

References Cited in the file of this patent

UNITED STATES PATENTS

| Number    | Name    | Date           |
|-----------|---------|----------------|
| 2,330,251 | Taylor  | Sept. 28, 1943 |
| 2,459,222 | Guthrie | Jan. 18, 1949  |